

## UNITED STATES PATENT OFFICE

2,397,262

## METALLURGICAL PROCESS

Charles H. Heist, Buffalo, N. Y., assignor to  
National Steel Corporation, a corporation of  
Delaware

No Drawing. Application March 30, 1943,  
Serial No. 481,147

4 Claims. (Cl. 75—133.5)

This invention relates to an improved process for making ferrosilicon.

In the present practice of making ferrosilicon or silvery iron a highly silicious ore is used together with a high hearth temperature. About one-third of the ore charge is normally Richmond ore or some other highly silicious ore. In the case of Richmond ore the silica runs about 40%. The coke burden is kept heavy in order to maintain a high temperature at the smelting zone. As the charge descends in the furnace the silica which is present mostly in the form of silicates melts and part immediately combines with limey substances to form slag. Of that portion which continues downwardly through the furnace the majority goes to the slag to satisfy the lime before reaching the smelting zone. Of that which does reach the smelting zone a portion, depending among other things upon the hearth temperature, is reduced to silicon which enters the iron. Silica is reduced in the presence of coke at a temperature of about 3200 and 3300° F.

Ferrosilicon usually runs from 7 to 15% silicon. An optimum proportion of silicon is 10% due to economic factors of blast furnace operation. In order to get 10% silicon into the iron under present operating conditions, a quantity of silica equal to about 22% of the ore charge must be available. When using a highly silicious ore the silicon, being present in the form of silicates, is melted at relatively low temperatures and is thus available for slagging and side reactions over a considerable part of the descent in the furnace. Additionally, a large body of these melted silicates are held in the burden by the blast and when the blast is reduced for tapping purposes this large body of liquid silicates rushes down through the smelting zone to join the slag without sufficient time for reduction in the smelting zone of some of the silica to silicon. This results in loss of silica to the slag besides the objectionable factors of a too highly silicious slag.

In view of the fact that silicon is reduced at

the proper temperature when it is in intimate contact with the incandescent coke, the applicant has conceived the idea of incorporating in the coke the amount of silica necessary to supply the silicon to the iron. By mixing fine sand with the coal to be coked the applicant has found that the resulting coke has silica thoroughly dispersed throughout its structure. This coke has improved metallurgical qualities, the presence of the silica mechanically held in the structure of the coke giving additional strength to the coke. It is well known that in its descent through the furnace the unconsumed coke retains its form right down to the point of combustion. Thus in the present process the silica is held within the interstices of the coke until the coke body reaches the smelting zone temperature and is consumed by combustion. At this point by maintaining the temperature between 3200 and 3300° F. the silica intimately held in contact with the coke is reduced to silicon and enters the iron. In the present process sufficient silica for fluxing is supplied by the ores used. If there is not sufficient silica present in the ores, sand may be added to the burden for fluxing purposes, the silica in the coke being destined for the iron. If the economics of the process demands that some highly silicious ores be used in the charge, less silica can be added to the coke or more lime used in the charge, the proportion of silica in the coke being maintained the same.

The applicant has found that by adding sufficient fine sand to the coke to bring the average silica content of the charged coke up to 15% any desired percentage of silicon in the iron between 7 and 15% can be achieved and therefore this percentage is preferred. In order to increase the amount of silicon going into the iron the proportion of coke charged is increased. The applicant has found that 10% silicon in the iron is still the most economical proportion under present operating conditions. To increase the silicon appreciably over this necessitates the use

of an amount of coke which makes the process uneconomic.

In producing his new metallurgical charging stock the applicant determines the amount of silica in the coke ash and adds sufficient fine sand to the coal charged to the coking process

resulting appears to be stronger than the coke product of the same coal without the silica.

Table 1 shows a mixture used in the prior practice of producing ferrosilicon in which 35% Richmond ore is charged. The coke used is 9.50% ash, giving 4.80%  $\text{SiO}_2$  in the coke.

TABLE 1  
*Stock analysis in per cent*

Ore per net ton pig iron 3,476 lbs. equals 1.74 tons net.

|                                                                |                         |     |                 |        |        |       |        |
|----------------------------------------------------------------|-------------------------|-----|-----------------|--------|--------|-------|--------|
| 10.00.....                                                     | 6,107                   | 9.7 | 2,352           | 43     | 346    | 1,140 | 152    |
| <hr/>                                                          |                         |     |                 |        |        |       |        |
| Total charge, lbs. $\text{SiO}_2$ , for 10.00% Si in pig 1,074 |                         |     |                 |        |        |       |        |
| Slag composition in lbs. per charge                            |                         |     |                 |        |        |       |        |
|                                                                | $\text{SiO}_2$          |     | 1,278           | 42.51  |        | 39.50 |        |
|                                                                | $\text{Al}_2\text{O}_3$ |     | 346             | 11.51  | 54.02  | 12.20 | 51.70  |
| Slag volume.....                                               | 49.25%                  |     | CaO.....        | 1,140  | 37.92  | 38.75 |        |
| Pounds stone per ton pig.....                                  | 754#                    |     | MgO.....        | 152    | 5.06   | 42.98 | 6.89   |
| Pounds slag per ton pig.....                                   | 986#                    |     | Add. 3%.....    | 91     | 3.00   |       | 2.66   |
| Pig iron tons per charge.....                                  | 3.05                    |     |                 |        |        |       |        |
|                                                                |                         |     | Total slag..... | 3,007  | 100.00 |       | 100.00 |
|                                                                |                         |     | Yield 50.18%    | 87.11% | 57.61  |       |        |

|                            |                                      |
|----------------------------|--------------------------------------|
| Pig iron analysis required | SiO <sub>2</sub> to bases equals .99 |
| C..... 2.00                |                                      |
| Si..... 10.00              |                                      |
| S..... .03                 |                                      |
| P..... .16                 |                                      |
| Mn..... .70                | Stone required 2,266 lbs             |

Document No. 87-11

so that the resulting coke product has 15% silica. No new problem is encountered in the coking process except that for the total coke product there will be about 10% less coking material resulting in shorter coking time and naturally less gas and by-products. The coke structure

Table 2 is a furnace mixture for use under present operating conditions which incorporates the present invention. No Richmond ore is used and the coke has 15%  $\text{SiO}_2$  including that in the ash.

TABLE 2  
Stock analysis in per cent

| Stock                           | Fe    | Phos  | SiO <sub>2</sub> | Mn    | Al <sub>2</sub> O <sub>3</sub> | CaO | MgO |
|---------------------------------|-------|-------|------------------|-------|--------------------------------|-----|-----|
| <i>Weight of charge, pounds</i> |       |       |                  |       |                                |     |     |
| Ore.....                        | 9,400 | 5,246 | 7.4              | 770   | 55                             | 88  | 23  |
| Coke.....                       | 7,157 | ----- | 1.4              | 1,074 | -----                          | 210 | 29  |
| Stone.....                      | 1,300 | ----- | .1               | 11    | -----                          | 641 | 59  |

Ore per ton pig iron 3,123 lbs. equals 1.56 tons net.

|  |       |     |       |    |     |     |    |
|--|-------|-----|-------|----|-----|-----|----|
|  | 6,026 | 8.9 | 1,855 | 55 | 208 | 693 | 81 |
|--|-------|-----|-------|----|-----|-----|----|

Total charge, lbs. SiO<sub>2</sub> for 10.00% Si in pig 1,194

|                                     |                                      |     |       |       |
|-------------------------------------|--------------------------------------|-----|-------|-------|
| Slag composition in lbs. per charge | SiO <sub>2</sub> .....               | 661 | 36.78 | %     |
| Slag volume.....                    | Al <sub>2</sub> O <sub>3</sub> ..... | 308 | 17.14 | 53.92 |
| Pounds stone per ton pig.....       | CaO.....                             | 693 | 38.57 | ----- |
| Pounds slag per ton pig.....        | MgO.....                             | 81  | 4.51  | 43.08 |
| Pig iron tons per charge.....       | Add. 3%.....                         | 54  | 3.00  | ----- |

Pig iron tons per charge..... 3.01 Total slag..... 1,797 100.00

Yield  $55.80 \div 87.07\% = 64.10\%$

Pig iron analysis required SiO<sub>2</sub> to bases equals .85

|               |
|---------------|
| C..... 2.00   |
| Si..... 10.00 |
| S..... .03    |
| P..... .15    |
| Mn..... .75   |

Stone required 1,290#

12.93

Percent Fe... 87.07

Table 3 shows a furnace mixture in which some Richmond ore is used. The coke used contains 15% SiO<sub>2</sub> including that in the ash.

cally to incorporate up to 15% of silicon into the iron and even higher percentages may be feasible with improved conditions of operation.

TABLE 3  
Stock analysis in per cent

| Stock ,                       | Fe    | Phos  | SiO <sub>2</sub> | Mn    | Al <sub>2</sub> O <sub>3</sub> | CaO   | MgO   |
|-------------------------------|-------|-------|------------------|-------|--------------------------------|-------|-------|
| 70% Hill Bessemer.....        | 56.46 | 0.033 | 8.93             | 0.12  | 0.37                           | ----- | ----- |
| 5 Amsden.....                 | 53.21 | .512  | 4.77             | .16   | 2.16                           | 1.11  | 0.54  |
| 7 1/2 Sinter.....             | 56.93 | .106  | 12.75            | .58   | 2.20                           | 2.57  | 1.60  |
| 7 1/2 (Crude) Portsmouth..... | 39.95 | .177  | 9.97             | 4.61  | 2.76                           | .21   | .25   |
| 10 Richmond.....              | 38.29 | .058  | 37.84            | .13   | 1.40                           | .34   | .44   |
| 200# Roll scale.....          | 73.30 | .036  | 70               | .51   | .21                            | ----- | ----- |
| 600# Borings.....             | 85.00 | .050  | 5.00             | .70   | -----                          | ----- | ----- |
| Silica-coke.....              | ----- | .020  | 15.00            | ----- | 2.94                           | .49   | .14   |
| HM stone.....                 | ----- | .011  | .84              | ----- | .79                            | 49.28 | 4.51  |

|                         |       |       |      |      |     |       |       |
|-------------------------|-------|-------|------|------|-----|-------|-------|
| <i>Mixture, percent</i> |       |       |      |      |     |       |       |
| Hill Bessemer.....      | 64.04 | 36.16 | .021 | 5.72 | .08 | .24   | ----- |
| Amsden.....             | 4.58  | 2.44  | .023 | .22  | .07 | .10   | .05   |
| Sinter.....             | 6.86  | 3.91  | .007 | .87  | .04 | .15   | .18   |
| (Crude) Portsmouth..... | 6.86  | 2.74  | .012 | .60  | .32 | .19   | .01   |
| Richmond.....           | 9.15  | 3.50  | .005 | 3.46 | .01 | .13   | .03   |
| Roll scale.....         | 2.13  | 1.56  | .001 | .01  | .01 | ----- | ----- |
| Borings.....            | 6.38  | 5.42  | .003 | .32  | .04 | ----- | ----- |

Average ore..... 100.00 55.73 .072 11.29 .57 .81 .27 .28

|                                 |       |       |     |       |       |     |     |
|---------------------------------|-------|-------|-----|-------|-------|-----|-----|
| <i>Weight of charge, pounds</i> |       |       |     |       |       |     |     |
| 8600 and 800 Ore.....           | 9,400 | 5,239 | 6.8 | 1,061 | 54    | 76  | 25  |
| Coke.....                       | 7,157 | ----- | 1.4 | 1,074 | ----- | 210 | 29  |
| Stone.....                      | 1,700 | ----- | .2  | 14    | ----- | 13  | 838 |

Ore per ton pig iron 3,124 lbs. equals 1.56 tons net.

|  |       |     |       |    |     |     |     |
|--|-------|-----|-------|----|-----|-----|-----|
|  | 6,018 | 8.4 | 2,159 | 54 | 299 | 892 | 113 |
|--|-------|-----|-------|----|-----|-----|-----|

|                                                                  |                                      |     |       |       |
|------------------------------------------------------------------|--------------------------------------|-----|-------|-------|
| Total charge, lbs. SiO <sub>2</sub> for 10.00% Si in pig, 1,193. | SiO <sub>2</sub> .....               | 966 | 41.26 | %     |
| Slag composition in lbs. per charge                              | Al <sub>2</sub> O <sub>3</sub> ..... | 299 | 12.77 | 54.03 |
| Slag volume.....                                                 | CaO.....                             | 892 | 38.11 | ----- |
| Pounds stone per ton pig.....                                    | MgO.....                             | 113 | 4.86  | 42.97 |
| Pounds slag per ton pig.....                                     | Add. 3%.....                         | 71  | 3.00  | ----- |

Pig iron tons per charge..... 3.01 Total slag..... 2,341 100.00

Yield  $55.73 \div 87.07\% = 64.02$

|                                                                  |  |  |  |  |  |  |  |
|------------------------------------------------------------------|--|--|--|--|--|--|--|
| Pig iron analysis required SiO <sub>2</sub> to bases equals .96. |  |  |  |  |  |  |  |
| C..... 2.00                                                      |  |  |  |  |  |  |  |
| Si..... 10.00                                                    |  |  |  |  |  |  |  |
| S..... .03                                                       |  |  |  |  |  |  |  |
| P..... .15                                                       |  |  |  |  |  |  |  |
| Mn..... .75                                                      |  |  |  |  |  |  |  |

12.93

Percent Fe... 87.07

It will be understood that the metallurgical charging stock of the present invention can be used in any process of incorporating silicon in a metal during reduction.

Using an oxygen enriched blast the process of the present invention can be utilized economi-

70 I claim:

1. In a process for producing ferrosilicon in a combustion type metallurgical furnace where iron ore is reduced and melted by the heat of combustion, charging iron ore containing silicon in combined form to the furnace, charging a flux-

ing agent to the furnace in sufficient quantity to remove the major portion of said silicon in slag form and charging silica and metallurgical coke to the furnace, the coke having the silica mechanically held in its structure in a quantity sufficient to supply the major portion of the silicon in the ferrosilicon product.

2. A process for producing ferrosilicon including from about 7% to about 15% silicon in a combustion type furnace wherein iron ore is melted primarily by the heat generated by the combustion of coke, said process comprising charging iron ore containing silicon in combined form to the furnace, charging a fluxing agent to the furnace in sufficient quantity to remove the major portion of said silicon in slag form and charging bodies consisting of about 15% silica and the remainder coke and incidental impurities to the furnace, the coke having the fine silica mechanically held in its structure in a quantity sufficient to supply the major portion of the silicon in the product; and burning said coke and causing said fluxing agent to remove the major portion of said combined silicon in slag form from said ore and causing the molten iron to combine with the silicon of said silica of said bodies in a quantity sufficient to produce said ferrosilicon product.

3. In a process for producing ferrosilicon including from 7% to 15% silicon in a combustion type furnace wherein iron ore is melted by the 30

heat of combustion, charging iron ore containing silicon in combined form to the furnace, charging a fluxing agent to the furnace in sufficient quantity to remove the major portion of said combined silicon in slag form and charging bodies consisting of about 15% silica and the remainder coke and incidental impurities to the furnace, the coke having fine silica mechanically held in its structure in a quantity sufficient to supply the major portion of the silicon in the ferrosilicon product.

4. A process for producing ferrosilicon in a combustion type furnace wherein iron ore is melted primarily by the heat generated by the combustion of coke, said process comprising charging iron ore containing silicon in combined form to the furnace, charging a fluxing agent to the furnace in sufficient quantity to remove the major portion of said combined silicon in slag form and charging bodies consisting of silica and coke to the furnace, the coke having fine silica mechanically held in its structure in a quantity sufficient to supply the major portion of the silicon in the product; and burning said coke and causing said fluxing agent to remove the major portion of said combined silicon in slag form from said ore and causing the molten iron to combine with the silicon of said bodies in a quantity sufficient to produce said ferrosilicon product.

CHARLES H. HEIST.